

C. A. KELLER.

PROCESS OF ELECTRICALLY TREATING, MELTING, AND REFINING METALS.  
APPLICATION FILED AUG. 12, 1902.

1,110,208.

Patented Sept. 8, 1914.

Fig. 1



Fig. 2



Witnesses:  
L. H. Groote  
Ernest Lundgren

Inventor:  
C. A. Keller  
by Agood & Co.  
Attys.

# UNITED STATES PATENT OFFICE.

CHARLES ALBERT KELLER, OF PARIS, FRANCE.

## PROCESS OF ELECTRICALLY TREATING, MELTING, AND REFINING METALS.

1,110,208.

Specification of Letters Patent. Patented Sept. 8, 1914.

Application filed August 12, 1902. Serial No. 119,885.

*To all whom it may concern:*

Be it known that I, CHARLES ALBERT KELLER, engineer, a citizen of the Republic of France, and resident of Paris, No. 3 Rue 5 Fignon, in France, have invented a certain new and useful Improved Process of Electrically Treating, Melting, and Refining Metals, of which the following is a specification.

10 The object of the present application is an electric process for melting and refining metals and other substances, particularly iron, cast iron and steel, applicable to various metallurgical operations, for instance, 1. 15 The introduction into one receptacle of one or several tappings coming from one or several melting apparatus, and there maintaining them at a temperature produced by electric current. 2. The refining of the material 20 or its mixture with others at any moment, 3. The melting and the mixture of metallic waste, particularly of iron and steel, 4. Refining of cast iron in the cupola itself after melting.

25 The process is based on the employment of an auxiliary chamber, generally a casting ladle, the contents of which can be easily and rapidly interposed in an electric circuit or be subjected to the action of the latter.

30 The annexed drawing gives an example of apparatus suitable for carrying out the process.

Figure 1 shows the arrangement when a casting ladle is used, Fig. 2 a vertical section 35 of a cupola as arranged for refining.

In Fig. 1 the casting ladle *a* rests by means of pivots or trunnions on one end of a beam *b*, the other end of which carries a counterweight *c* intended for balancing the 40 ladle and its charge; this beam is carried by a truck *d*, which can be moved on rails. This arrangement allows of bringing the ladle *a* to the proximity of a melting furnace to receive the successive tappings or to the 45 proximity of each of a series of furnaces to receive in succession the tappings from such furnaces; it also permits of bringing the same ladle under an apparatus comprising vertical electrodes *e*, *e* supported by chain tackle so as to raise or lower them into the ladle for the requirements of the operation 50 as hereinafter described.

In Fig. 2 the cupola *f* is provided with a fore-hearth *g* to receive the molten metal 55 and above which is arranged a group of ver-

tically movable electrodes *e*, *e* similar to those previously described.

Taking the first case into account, the ladle *a*, having a refractory lining, does not form part of the electric circuit; the current 60 enters and leaves through vertical electrodes *e*, *e*, arranged above it; these electrodes can be regulated and each constitutes in effect a separate furnace, and in practice I employ more than two electrodes for each pole; this 65 permits of always being able to replace an electrode at work without interrupting or disturbing the course of the operation. If only one electrode were provided its removal would cause the breakage of the circuit. On 70 the other hand, if each pole carries a minimum of two electrodes, it will be possible to remove one of them and this would only result in an increase of current in the remaining electrodes. As an example, the manu- 75 facture of iron or of steel will be described.

The metal contained in the ladle can be easily put into the electric circuit through the suitable lowering of the electrodes into the bath. The ladle is carried on a truck 80 adapted to be moved so as to be brought successively under the tapping orifices of furnaces of the same battery. This arrangement will be particularly useful with the battery of electric furnaces, as the respective output of this kind of apparatus is less than that of blast furnaces or metallurgical melting furnaces of the ordinary kind. After each tapping or set of tappings the molten material contained in the ladle is 85 introduced into the electric circuit and the reheating is effected by a current of suitable strength, regulatable as required. By these means the metal is maintained at the required temperature; 90 the quantity of heat necessary for this purpose will simply compensate that quantity lost by radiation. The slag which will have probably been tapped with the metal from the furnaces is removed in convenient quantity from the ladle so as not to be superfluously reheated. This removal is effected by simply tilting the ladle. The electric current is interrupted when the ladle has again to be placed under the openings of the melting furnace or furnaces; to receive a further tapping or tappings and the reheating, if required, then takes place as described 105 above. By this process a new method of working is realized; very large castings can 110

be made with apparatus, the practical output of which is much less than the weight of these pieces. The temperature of the molten metal can be easily regulated and the metal 5 remaining in the ladle after tapping will not be wasted as often happens, as it can be kept hot until mixed with other tappings; the founder can therefore estimate the amount of metal required for the filling up 10 of large molds without fear of waste resulting from too high an estimate, which leads him sometimes to under-estimate and to spoil castings through insufficiency of metal in the ladle.

15 To refine or make additions to the metal collected in the ladle it is introduced into the electric circuit, and the removal of slag proceeded with if required, as already described; the current is then regulated so 20 as to considerably reheat the metal to be refined, and the necessary additions are then made to obtain the required quality. For example, steel can be manufactured with cast iron from ordinary cupolas by refining this cast-iron by the addition of oxid 25 and, just as in the Martin furnace, one can desulphurize, dephosphorize and deoxidize. This process therefore permits of transforming an ordinary foundry into a steel 30 foundry. This process of refining or mixing can also be employed for the metal coming from ordinary furnaces as well as for that from electric furnaces.

The process can also be easily applied to 35 the melting and mixture of steel and iron waste which it may be required to remelt, owing to the extreme facility it offers of taking samples, because of the continuous access it permits to the metal in the ladle. 40 For this purpose a certain quantity of molten metal (iron, steel or cast iron) is first introduced into the ladle, and a certain quantity of ore which covers over the metal. The electric current is then passed 45 into the ladle and the operation having thus commenced, pieces of metal to be remelted and mixed are introduced into the liquid layer. These pieces of metal could not be placed in circuit in the empty ladle on account of their weak electrical resistance, or 50 an electric current of a strength inadmissible in practice would have to be used and which would cause large fluctuations in the operation. With this process, which utilizes 55 the usual strengths of current employed in electric melting, the operation is rendered normal and effective by throwing the respective pieces of metal to be melted into the initial metal bath formed in the ladle 60 as described. Under these conditions, the electric working of the apparatus is in no way disturbed and when the melting is complete, the additions can be made and the operation effected according to the usual 65 method of mixing and refining of metals.

in the metallurgy of iron, the second melting effected as described corresponds to the actual manufacture in the crucible.

The process above described also permits of transforming the ordinary remelting cupolas into mixed furnaces for obtaining cast iron or steel. As known, some cupolas have a fore-hearth into which the manufactured cast iron arrives; it is this basin which will replace the ladle, for putting this process 70 into practice, which will permit of manufacturing steel with existing apparatus for the manufacture of iron. In this form of application, there is arranged over the existing or specially constructed fore-hearth 75 (as has been described with reference to Fig. 2) a group of vertical electrodes *e*, *e*, which are lowered into it, after receiving the cast iron, and the refining is effected as previously described, after removal of slag. 80 During tapping the electrodes can be removed or not, and the operation is proceeded with as usual.

It is evident that for the refining operations in the case of ladles as well as in cupolas neutral, acid or basic linings are employed, as the case may be.

I have in some of the claims referred to "iron," by which I desire to be understood either cast iron, wrought or ingot iron or 95 steel.

I claim:

1. The process of electrically treating, melting and refining metals, consisting in moving a suitable receptacle to two or more 100 furnaces and collecting the products of metallurgical operations in said receptacle, lowering electrodes into the collected products while in a state of fusion, and subjecting the said products to the action of an 105 electric current of sufficient strength to further heat and refine them.

2. In the treatment of steel, the process of mixing the products from a number of furnaces, which consists in introducing them 110 in a molten condition into a single receptacle, and maintaining the mass molten in said receptacle by heat from an electric current, removing portions only of the composite molten contents of the receptacle 115 without entirely emptying the same, and successively replenishing the receptacle with fresh additions.

3. In the treatment of steel, the process which consists in introducing the steel in a 120 molten condition into a receptacle, and maintaining it molten in said receptacle by the heat from an electric current, said process being carried on without the use of a flame or other oxidizing method of heating, 125 whereby desulphurization and conservation of the oxidizable additions are favored.

4. In the art of converting cast iron or the like into high-grade or "crucible" steel, the method which consists in transferring steel 130

produced in any ordinary furnace or operation into an electric furnace, and finally treating the steel in said electric furnace to deoxidize it and making any desired addition thereto.

5. In the art of converting cast iron or the like into high-grade or "crucible" steel, the method which consists in transferring steel produced in any ordinary furnace or 10 operation into an electric furnace, with removal of the superfluous slag, and finally transforming it in said electric furnace into the desired product.

15. In the art of electrically treating, melting or refining metals, the method which

consists in moving a receptacle to an apparatus supplying molten metal, charging metal into said receptacle, moving the charged receptacle into proximity to electrodes, and adjusting said electrodes and establishing an electric current of sufficient strength through the charge, thereby heating it to the desired temperature. 20

In testimony whereof I have signed my name to this specification in the presence of 25 two subscribing witnesses.

CHARLES ALBERT KELLER.

Witnesses:

JULIAN CAVERUE,

PAUL BACARD.